

Patented May 28, 1929.

1,714,679

# UNITED STATES PATENT OFFICE.

DONALD C. LEE, OF SPOKANE, WASHINGTON.

## ALLOY.

No Drawing.

Application filed November 17, 1926. Serial No. 149,006.

My present invention relates to an improved alloy for use as anti-friction metal and adapted especially for bearings of rotary journals as well as for sliding machine-elements. The invention consists in an alloy as an article of manufacture having as its major portion or element, brass that is united with Babbitt metal, lead, or pewter, as desired, by the use of a flux during the alloying process. In the production of the alloy in connection with brass as the major element or metal, the brass is subjected to a milling process by means of which it is reduced to a finely comminuted grain or coarse powder. The metal with which the brass is to be united is first reduced to a molten state and then the milled or powdered brass is added thereto, together with a flux for uniting the elements of the alloy into a homogeneous whole.

Thus as an exemplification of my invention in the uniting of brass and Babbitt metal, the Babbitt metal may form twenty per cent of the final product or alloy.

The brass which will form the remaining eighty per cent of the final product or alloy may be made up of the following metals, in copper 20 parts, zinc 3 parts and tin 3 parts. The proportion of the brass and babbitt may be varied, and the ratio of metals in the brass and Babbitt metal may also vary.

The Babbitt metal is prepared in a crucible by the application of the necessary heat in any usual manner, and brought to a molten state.

The brass is finely comminuted by suitable mechanical means. A flux is utilized for uniting these prepared elements during the alloying process. One formula for the flux or solution may comprise the following materials in the proportions stated:—

|                         |           |
|-------------------------|-----------|
| Muriatic acid           | 1 gallon  |
| Zinc                    | 3 pounds  |
| Blue vitriol (crystals) | 12 ounces |
| Resin                   | 21 ounces |

This flux is separately prepared by first placing the muriatic acid in a suitable container and adding thereto a supply of zinc strips as rapidly as may be for the dissolution of the zinc by chemical action in the acid.

While the acid is attacking and dissolving the zinc strips a supply of blue vitriol (crystals) is added to this mixture, which is stirred or agitated in usual manner to assist in the dissolution and the formation of a homoge-

neous solution. Additional quantities of zinc are added as rapidly as the mixture will absorb the zinc. At this stage the resin is added to the solution and the whole mass is continuously stirred or agitated until the chemical changes cease in the solution. The top of the solution is then skimmed off to remove any scum and after cooling, the solution or flux is ready for addition to the metals which will form the alloy.

The brass as previously prepared and in comminuted form is added to the molten Babbitt metal contained in the crucible and the solution as above prepared is preferably atomized in proper devices and added simultaneously to the molten metal with the brass shavings or powder. During the introduction of the brass and flux to the molten Babbitt metal, the mass while heated to the required temperature, is stirred and agitated by suitable means until the constituent parts of brass, Babbitt metal and the solution or flux are thoroughly united and form a molten mass. The final product is thus composed of the various elements of Babbitt metal and of brass, alloyed together, in approximately the proportions of 80% brass and 20% Babbitt metal. The ratio of copper and zinc in the brass may be as three to two, and the proportions in the Babbitt metal may be tin 83%; copper 9% and antimony 8%.

The proportion of the flux used to the alloy and the ratio of parts or metals in the brass and Babbitt metal may vary or differ with the desired degree of hardness of the finished product or alloy. If a journal bearing is to be formed, the united alloy as molten metal may be poured from the crucible directly into a mold for the formation of the desired bearing structure. Or the molten metal may be poured from the crucible into desired shapes or castings for subsequent use.

I find that the brass, Babbitt metal and flux unite readily and perfectly, and the production of anti-friction metal is thus accomplished at a comparatively inexpensive cost. The alloy is of such tenacity that when molded in a journal bearing for instance, it eliminates danger of cracking or breaking, and insures durability not only for bearings for rotary journals, but also for machine elements having sliding frictional contact. While the alloy produces but slight friction to the moving parts, it is of sufficient hardness to reduce abrasions and wear to a minimum without cutting or injuring the frictionally engaged

parts. The alloy is of a sufficiently high melting point as to be infusible under conditions where considerable heat is generated by friction, as in a journal bearing.

5 Having thus fully described my invention, what I claim as new and desire to secure by Letters Patent is:

10 1. An anti-friction metal comprising an alloy of approximately 80% brass and 20% Babbitt metal.

15 2. The process of preparing an anti-friction metal which consists in comminuting brass, reducing Babbitt metal to a molten state, adding the comminuted brass to the molten Babbitt metal, adding a flux-solution, maintaining the mixture in a molten state and agitating it to form a uniform alloy.

3. The process of preparing an anti-friction metal which consists in reducing Babbitt metal to a molten mass, adding comminuted brass to the molten metal, atomizing a flux-solution to the mixture and stirring it to form an alloy, and cooling the final product.

4. The process of preparing an anti-friction metal which consists in comminuting brass, reducing Babbitt metal to a molten state, adding the comminuted brass to the molten Babbitt metal, adding a flux-solution comprising muriatic acid, zinc, blue vitriol and resin in suitable proportions, maintaining the mixture in a molten state and agitating it to form a uniform alloy.

In testimony whereof I affix my signature.

DONALD C. LEE.